

1,291,253.

C. J. THATCHER,  
DIAPHRAGM OR SEPARATOR,  
APPLICATION FILED MAR. 22, 1915.

Patented Jan. 14, 1919.



WITNESSES:

Sally O. Gudzak  
Arthur Worscheck

INVENTOR

Charles J. Thatcher

# UNITED STATES PATENT OFFICE.

CHARLES J. THATCHER, OF NEW YORK, N. Y.

## DIAPHRAGM OR SEPARATOR.

1,291,253.

Specification of Letters Patent. Patented Jan. 14, 1919.

Application filed March 22, 1915. Serial No. 16,285.

*To all whom it may concern:*

Be it known that I, CHARLES J. THATCHER, a citizen of the United States, and a resident of New York city, in the county of New York and State of New York, have invented certain new and useful Improvements in Diaphragms or Separators, of which the following is a specification.

This invention relates to improvements in separators or diaphragms for use in separating two liquids from one another, as, for example, in an electrolytic cell.

The object of the invention is to provide diaphragms of ample mechanical strength which shall also be capable of withstanding the action of corrosive electrolytes—particularly of hot, alkaline or acid liquids—but nevertheless be so constructed as to permit of uniform distribution of a superior ion transmitting medium, which medium shall at the same time, serve to eliminate transfusion of anolyte and catholyte liquids into one another.

The drawing illustrates an enlarged section of my improved diaphragm or separator and shows the substantially uniform size and distribution of the voids *a, a*, and the character of the grains of material *b, b*, and their bonding, fused or other joints at the points of juxtaposition, *c. c.*

For the purposes of my invention I prefer to use plates, cylinders or other vessels, composed of substantially uniform grains of mineral or other materials cemented together as by incipient fusion. "Filtros," composed of grains of sand or crystalline silica, and "alundum," composed of granular aluminum oxid, are good examples of such materials. They are admirably suited to the purpose of my invention because they contain a high percentage of voids, which are uniform in size and uniformly distributed throughout the material. These characteristics, together with their mechanical strength, make such materials admirable for the construction of diaphragms for the most varied kinds of large electrolytic cells and vats.

These materials of course are unaffected by acids. They have certain defects, however, which militate against their general use for diaphragms. They are slowly disintegrated and dissolved by hot, strongly alkaline liquids; and they are so porous that the anolyte and catholyte mix with considerable rapidity, even through the densest

grades of such materials which it has been possible to produce. No method of overcoming the first of these defects has been practically successful. Attempts to obviate the excessive permeability to liquids, by making the materials from extremely fine grains of silica or crystalline alumina, have only resulted in increasing the electrical resistance without materially reducing the transfusion of anolyte and catholyte into one another through the diaphragm, which transfusion the latter is designed to eliminate.

To obviate the disadvantages of the aforesaid materials for diaphragms I proceed as follows:

For preparing diaphragms or separators for use in electrolytic cells of any kind or in similar apparatus, I use preferably coarsely grained plates or cylinders, *e. g.*, "filtros" or "alundum" having coarse, more or less uniform grains cemented together substantially only at their points of juxtaposition. Such coarsely grained filtros or alundum plates, etc., are more porous, and contain a larger percentage of voids. Their voids are more uniform in size and more uniformly distributed throughout the material than in the case of the finer grained materials which have hitherto been selected for diaphragms, in order to reduce, as far as possible, the undesirable transfusion therethrough of the anolyte and catholyte into one another. The drawing, which shows a somewhat enlarged section of my improved diaphragm, illustrates the foregoing description of the class of materials which I preferably employ.

I will describe first the preparation from such materials of diaphragms intended to be used only for alkaline liquids.

The porous plate or vessel, preferably dry or nearly so, is first saturated with a solution of a salt of a metal which is capable of forming gelatinous hydrates, insoluble in caustic alkalis. Magnesium is an example of such a metal, and the porous material may be soaked in a solution of magnesium sulfate, for example, the solution being preferably quite concentrated.

After the porous material has become well saturated with this solution, I remove it therefrom, and then immerse it in a solution of a hydrate such as sodium hydroxid. A ten per cent. solution suffices, but more dilute or more concentrated solutions may be employed. The porous material should

be allowed to remain in the caustic soda solution for a suitable time—until the alkaline solution has had opportunity to penetrate into all parts of the porous material—which time, of course, will vary with the dimensions of the material. The penetration of the caustic soda solution by diffusion to the innermost parts of the porous material will not be rapid because all of the surface interstices and pores of the material become filled immediately with a gelatinous medium, consisting of hydrate of magnesium, which cannot be washed out of the pores but effectually and permanently fills them, thereby making the porous material substantially impermeable to liquids. Ions, however, will migrate through the moist, gelatinous material as readily as through water.

20 After this precipitation of the gelatinous substance, the impregnated material may be immersed for some hours in water to allow the sulfates or other salts of the alkali metals to diffuse out, if that is thought necessary. The plates are then ready for use; they will be moist because of the water retained by the gelatinous hydrate, and should be preferably maintained in a moist condition so that the gelatinous material 30 will not shrink up by drying and cease to fill the pores. In some instances, however, later moistening of the diaphragm material and thereby of the gelatinous substance contained therein may cause the gelatinous substance to swell up and again effectually close the pores of the diaphragm material. But to prevent such drying and shrinking of the gelatinous substance, as for example during shipment of the diaphragms, calcium chlorid, caustic soda, or other hygroscopic substances may be applied to the surfaces or introduced into the interior of the impregnated, diaphragm material, as by immersing the latter in a solution of the specified hygroscopic substances, 45 and with the result that the plates will permanently retain their moist condition. These hygroscopic substances, of course, if they are undesirable, can be subsequently washed out before use, but the impregnated material thereafter should be preferably maintained in a moist condition.

It will be understood that care should be taken to have all parts of the porous material equally saturated with the magnesium sulfate solution, and then with the alkali solution, and that these treatments may be effected in reverse order and also while the diaphragm material is in place in the cell in which it is to be used. Electrolysis, using the magnesium sulfate solution as anolyte and the solution of the hydrate as catholyte, will of course facilitate precipitation of the gelatinous hydrate in the pores of the intervening diaphragm material where the

migrating magnesium and hydroxyl ions meet.

By thus precipitating hydrates, which are practically insoluble in alkalis, in the pores of materials such as "filtros" or "alundum," 70 they become more resistant to alkaline liquids, which effect it is one of the objects of my invention to attain. The gelatinous substance, deposited in the pores of the diaphragm material, does not hinder 75 electrolytic conduction by migrating ions, but it does prevent the access of fresh portions of the caustic alkaline liquid to the diaphragm material; so that the solvent action of the caustic liquid is diminished to 80 the point of elimination, being restricted to that exerted by the metal and hydroxyl ions introduced into the plate by electrolysis.

Furthermore, in the case of silicious materials such as "filtros", as soon as there is any solution, by the caustic alkali, of silica at any point, the resulting alkaline silicate solution immediately reacts with the adjacent magnesium hydrate forming, *in situ*, dense, 85 90 gelatinous magnesium silicate, as a coating around the solid particle of silica which had been attacked, and thereby serves to eliminate further access to and solvent action upon the silica by the caustic liquid. 95 "Filtros" or similar granular materials, when thus treated, may be used continuously for long periods in hot, alkaline liquids without serious disintegration. Such impregnated diaphragms have an electrical 100 resistance, which, providing they contain 50% of voids for example, is only about twice as great as a body of the electrolyte having the same dimensions as the plate. By volume the diaphragms are composed of 105 50%, for example, of a good conducting, gelatinous material, which is practically impermeable to liquids and which is uniformly distributed throughout the diaphragm, being held in place, so to speak, by 110 the uniform, coarsely granular frame work of the diaphragm material. By thus combining uniformly and highly porous granular material with a good conducting gelatinous medium I am able to produce 115 diaphragms which offer little resistance to the passage of the electric current; which conduct the current uniformly throughout and which are practically impermeable to liquids; and which, in case magnesium hydrate is used as a gelatinous medium, are not measurably disintegrated by corrosive, alkaline liquids.

Diaphragms made by the previously described process cannot be used in ammoniacal nor in acid solutions, both of which of course dissolve the gelatinous magnesium or other hydrate.

In constructing diaphragms for use in solutions of ammonia or its salts, I impreg- 130

nate the plate with gelatinous hydrate of alumina or with the hydrate of some other metal which is insoluble in ammoniacal solutions. This is accomplished by carrying out the treatments previously described, substituting a soluble salt of alumina for the magnesium sulfate and a solution of ammonium hydroxid for the caustic soda solution. The result will be a diaphragm composed of uniformly distributed, gelatinous aluminum hydrate, embedded in coarse grained silica or aluminum oxid and, which will not be attacked by ammoniacal solutions, and will moreover possess all the advantageous properties of the improved diaphragms heretofore described.

Diagrams which are to be used in either acid or alkaline liquids or with an acid liquid on one side of the diaphragm and an alkaline on the other, are similarly produced by impregnating "filtros," "alundum," or similar granular material with gelatinous magnesium silicate or equivalent gelatinous silicates which are not dissolved by acids or alkalis. It will be readily understood that this can be accomplished by carrying out the treatments previously specified for the production of diaphragms impregnated with magnesium hydrate, substituting a more or less concentrated solution of water-glass for the caustic soda specified for use in that treatment. In this case it would be preferable to first saturate the suitable "filtros" or "alundum" material with the sodium silicate solution and then with the magnesium or other metallic salt solution. Subsequent washing and addition of hygroscopic substances may be employed, substantially as before described. Such impregnated diaphragms will have all of the novel characteristics previously set forth and in addition thereto be capable of use for prolonged periods in either acid or alkaline liquids, or in both. As soon as solution of silica by caustic soda, for example, begins at any point, the resulting sodium silicate reacts with the magnesium silicate to form a more silicious magnesium silicate or double silicate of sodium and magnesium, and with the result that the diaphragm material does not waste away and that further solution is substantially eliminated.

Diaphragms suitable for prolonged use in acid liquids, having a uniform and maximum permeability to migrating ions but not permeable to liquids may be similarly constructed by impregnating "filtros," "alundum" or similar uniformly, granular materials with gelatinous hydrate of silica, which is insoluble in acids, as are also the porous materials specified. It will be also understood that this impregnation can be effected by immersing such materials, first in a wa-

ter-glass solution of considerable strength, and then in diluted sulfuric or other acids, which will cause a precipitation, within the voids, of gelatinous silica hydrates with the results hitherto specified. Subsequent washing out of sodium sulfate, etc., may be resorted to if that seems desirable; and by thereafter introducing or by retaining some sulfuric acid within the gelatinous medium it will be hygroscopic and the drying out of the gelatinous material which is undesirable will be avoided.

The diaphragms previously described, prepared by impregnating "filtros," "alundum," or other uniformly granular materials with magnesium or aluminum or other hydrates, or with magnesium silicate or silica hydrates, may of course be used with neutral liquids, proper care being taken to select a gelatinous impregnating medium which is adapted to the liquid or liquids in which it is being used. A diaphragm impregnated with magnesium hydroxid should not be used in a neutral solution containing ammonia salts, for example, because the latter exert a solvent action upon magnesium hydrate.

I claim:

1. An electrolytically good conducting, substantially non-filtering medium suitable for diaphragms, consisting of a non-cellular, granular, structure and of a gelatinous impregnating material.

2. An electrolytically good conducting, substantially non-filtering medium suitable for diaphragms, consisting of a non-cellular, granular structure containing a high percentage of voids, and of a gelatinous medium in said voids.

3. An electrolytically good conducting, substantially non-filtering medium suitable for diaphragms, consisting of a non-cellular granular structure containing substantially uniformly distributed voids, and of a gelatinous medium in said voids.

4. An electrolytically good conducting, substantially non-filtering medium suitable for diaphragms, consisting of a non-cellular, granular silica structure and of a gelatinous impregnating material.

5. An electrolytically good conducting, substantially non-filtering medium suitable for diaphragms, consisting of a rigid, porous, non-cellular structure composed of cohering grains of silica, and of a gelatinous silicious impregnating material.

Signed at New York city, in the county of New York and State of New York, this 20th day of March, A. D. 1915.

CHARLES J. THATCHER.

Witnesses:

ARTHUR WORISCHKE,  
LAURA E. SMITH.